

## UNITED STATES PATENT OFFICE

1,931,368

## TREATMENT OF NITROCELLULOSE DOPE

Linton C. Amberson, Edensburg, Pa.

No Drawing. Application November 24, 1931  
Serial No. 577,166

8 Claims. (Cl. 134—79)

The present invention relates to treating nitrocellulose dope (i. e. viscous solutions of nitrocellulose in suitable volatile organic solvents) such as is used for coating airplanes, balloons and similar fabrics, and the object is to improve the dope, and to improve the film of material left when the dope is applied to the said fabric and dried, particularly rendering the dried coating substantially non-inflammable, or at least of a low degree of inflammability as compared with the highly inflammable nitrocellulose.

It is of course understood that the dopes now on the market, made by different manufacturers have different chemical compositions, that is to say the proportion of nitrocellulose therein and the proportion of plasticizing agents and the specific character of the solvents employed, are all more or less variable.

In accordance with the present invention I treat a solution of nitrocellulose, for example a nitrocellulose dope which may be any one of those now on the market. To the solution of nitrocellulose, for example nitrocellulose dope, I add an acid solution of zinc salt, preferably zinc chloride dissolved in commercial strong hydrochloric acid (1.2 gravity) to substantial saturation. I prefer to use about 2 volumes of this zinc salt solution to 1 volume of the nitrocellulose dope. These two materials are well mixed together, which produces coagulation of the nitrocellulose, and the liquids are thoroughly mixed, while being poured together. The cellulosic compound is thereby converted into the insoluble condition, as a more or less stringy mass. This will be of a grayish color, and apparently contains, in addition to the cellulosic compound, zinc compounds and some acid. This stringy mass is then washed one or more times with a solution of magnesium sulfate, for example a solution containing about 6 to 10% of Epsom salts (crystallized magnesium sulfate). This turns the stringy mass to a practically white condition, and washes out the remaining free hydrochloric acid. One or more washings with the magnesium sulfate will be sufficient, and it is advisable to test at this stage to see that the cotton-like stringy mass is substantially acid free. This can be tested with litmus paper or by adding a little sodium bicarbonate which would cause considerable effervescence if free acid is still present. The mass is then washed with water one or more times, and is allowed to stand and drain for the excess water to drain away. It is not necessary at this stage to dry the material, but most of the water can be separated out by gentle pressure.

At this stage a softener or plasticizing agent can be added, to the amount of one-half ounce per gallon of the washed mass, which will amount to about one-half per cent of the weight of the mass under treatment. As suitable plasticizing agents, castor oil and tri-cresyl phosphate are mentioned. Other similarly acting softeners can be employed.

The cellulosic material and softener are worked together, for example by a stirring and kneading action, during which operation a further amount of the water in the mass may separate out mechanically, which can be discarded. Then, without drying, the mixture of cellulosic compound and castor oil (or other softener) is added to another three volumes of the original dope. To make clear the matter of proportions, assuming one gallon of the original dope was used in a particular case, the resulting cellulosic material and softener would be then added to three gallons of the untreated dope. This amount will readily dissolve in the dope, and thinners such as alcohols or acetates, or other diluents, can then be added to obtain the desired consistency.

It will of course be understood that the invention is in no sense restricted to dope to be applied to fabrics, but can be applied in a similar manner to various other nitrocellulose solutions. The final mixture of cellulosic compound and softener can be dissolved in a dope or in any other nitrocellulose solvent.

In some cases it is advisable to dissolve the cellulosic material from one volume of dope, in less than three volumes of untreated dope, for example two volumes or two and one-half volumes. In some cases this material could be added to more than three volumes of the dope.

I claim:—

1. A process which comprises treating a solution of nitrocellulose with an aqueous acid solution of a zinc salt to produce precipitation of the nitrocellulose, then drawing off the acid liquid, washing the residue with an aqueous solution of a magnesium salt, and finally washing same with water; adding a plasticizer to the wet residue and working the same together with further separation of water, and dissolving such product in a liquid containing volatile solvents.

2. A process as in claim 1, in which the acid aqueous solution of zinc salt is a substantially saturated solution of zinc chloride in hydrochloric acid, and in which the aqueous solution of a magnesium salt is a 6 to 10% solution of Epsom salt in water.

3. A process which comprises treating a nitro-

cellulose dope with more than its own volume of a substantially saturated solution of zinc chloride in concentrated aqueous hydrochloric acid, to cause a coagulation of the nitrocellulose, wash-  
5 ing the latter with a dilute aqueous solution of Epsom salt, thereafter washing same with water, and dissolving the product in a pyroxylin solvent.

4. A process which comprises treating a nitro-  
10 cellulose dope with more than its own volume of a substantially saturated solution of zinc chloride in concentrated aqueous hydrochloric acid, to cause a coagulation of the nitrocellulose, washing the latter with a dilute aqueous solution of Epsom salt, thereafter washing same with water, mixing the residue with a small percent-  
15 age of a plasticizing agent, and dissolving the mixture in a liquid containing a nitrocellulose solvent.

5. A process which comprises treating a nitro-  
20 cellulose dope with more than its own volume of a substantially saturated solution of zinc chloride in concentrated aqueous hydrochloric acid, to cause a coagulation of the nitrocellulose, washing the latter with a dilute aqueous solution of Epsom salt, thereafter washing same with water, and thereafter dissolving the residue in a  
25 nitrocellulose dope.

6. A process which comprises treating a nitro-

30

80

85

90

95

100

35

105

40

110

45

115

50

120

55

125

60

130

65

135

70

140

75

145

cellulose dope with more than its own volume of a substantially saturated solution of zinc chlo-  
ride in concentrated aqueous hydrochloric acid, to cause a coagulation of the nitrocellulose, wash-  
ing the latter with a dilute aqueous solution of Epsom salt, thereafter washing same with water, mixing the residue with about one-half per cent of a liquid plasticizing agent and there-  
after dissolving the mixture in a nitrocellulose dope, to produce a dope which, upon being ap-  
plied and dried, is of reduced inflammability.

7. A process which comprises treating a nitro-  
cellulose dope with more than its own volume of a substantially saturated solution of zinc chlo-  
ride in concentrated aqueous hydrochloric acid, to cause a coagulation of the nitrocellulose, wash-  
ing the latter with a dilute aqueous solution of Epsom salt, thereafter washing same with water, mixing the residue with about one-half per cent of a liquid plasticizing agent and there-  
after dissolving the mixture in a nitrocellulose dope and adding more pyroxylin solvent as a thinner, to produce a dope which, upon being ap-  
plied and dried, is of reduced inflammability.

8. Nitrocellulose dope having the properties 100  
of the product of claim 7.

LINTON C. AMBERSON.